

## UNITED STATES PATENT OFFICE

EDMONDSON SPENCER, OF CALCUTTA, BRITISH INDIA

## PROCESS FOR SEPARATING OR EXTRACTING CELLULOSE OR PAPER PULP

No Drawing. Application filed February 10, 1928, Serial No. 253,311, and in British India May 28, 1927.

This invention relates to processes for the separation or extraction of cellulose or paper-pulp from vegetable matter containing the same, and has for its object modifications of the processes which are calculated to increase the yield of cellulose and the quality of the product.

In the digestion of materials to produce cellulose and paper pulp it is usual to increase the activity of the digesting liquors towards the final stages of the digestion in cases where the digestion is carried out on the semi-continuous, progressive, step-by-step or the cascade system; whereas in the ordinary or overhead process, the activity cannot increase as the digestion proceeds, since the proportion of active reagent is continually diminishing. In the overhead process a given amount of caustic is added and the strength of active caustic progressively diminishes towards the end of the digestion. This together with the fact that all the products of decomposition are present to the end of the process constitutes the main weakness of the over-head process. To surmount these two difficulties the cascade process aims at removing the products of decomposition in successive stages and in replacing the liquors with fresh solutions relatively stronger in active alkali and relatively weaker in products of decomposition. By this means the digestion time is shortened very considerably. The largely increased activity of free caustic in the latter stages may however result in a partial destruction of a portion of the cellulose fibre, and to guard against this it may be advisable to have the greatest strength of active alkali not at the last digestion stages but at some stage earlier in the digestion at a lower pressure and with more of the non-cellulosic material still to be removed, or, alternately, when using mixed liquors (such as caustic and sulphites and/or sulphides, which latter exert a protective action), a similar result is obtained by proportioning the liquors added in such a way that the hydrolysis is prevented by having a relatively greater proportion of the more protective or less severe reagents in the final stage of the digestion.

The invention relates mainly to processes wherein mixed digestor liquors are used in at least part of the digestion period and wherein the process of digestion is carried out in successive stages, but it is not restricted to use with mixed digestor liquors alone.

It is known that sodium mono-sulphite  $Na_2SO_3$  is not so severe in its action on cellulose fibres at raised pulping temperatures as ordinary caustic is.

Also it is known that sulphide liquors are somewhat similar to sulphite liquors in this respect that they are not so active as caustic in attacking the more easily resolvable celluloses.

When using a mixed digestor liquor, such as a mixture of caustic soda, sulphite and/or sulphide it may be advantageous to have certain of these chemicals in solution in separate tanks and add certain limited quantities to the digestors according to a preconcerted plan. For example, sodium sulphite and sodium sulphide being known to exert a protective action on the cellulose fibre in reducing the hydrolyzing effect it may accordingly be advantageous to have a relatively large proportion of these reagents in the final (drastic) stages of the treatment and a relatively larger proportion of the caustic soda in the preceding stages of the process.

According to one part of this invention the composition of the digesting liquors is altered as the digestion proceeds. The alteration may take place at any stage but more particularly towards the final stages of the digestion.

According to this invention a certain amount of protection may be afforded to the fibre reducing hydrolysis, by manipulating and even by actually reducing the digestion pressures in the final stage of the process. By manipulating the composition of the digesting liquors and the pressure at which the process operates, by raising the pressure gradually or in steps in the earlier stages and by holding the pressure constant towards the end of the cook combined with a variation in the liquor constitution or proportions, and even by reducing the final pressures below the maximum ones used when found desir-

60

65

66

70

75

80

85

90

95

100

able, an increased yield of cellulose and an improved pulp may be obtained.

- The invention is applicable to any digestion process for the purposes explained 5 worked on a semi-continuous, progressive, step-by-step or cascade system or to a process wherein the pressure heretofore or generally has been or is held constant or is raised gradually or in steps as the cooking proceeds, but 10 wherein the free caustic concentration or the active digesting liquor concentration is raised also as the process proceeds preferably either in steps or at some point or points in the process.
- 15 It is however more particularly applicable to processes of the type described and claimed in application Serial No. 253,310, filed February 10, 1928, and Patent No. 1,690,954, dated November 6, 1928, wherein the pulp 20 forming material is subjected in a digester to successive treatments at increasing pressures and with increasing active liquor concentrations in a step-up pressure-free-caustic-concentration gradient.
- 25 The invention accordingly comprises a process for separating or extracting cellulose or paper-pulp from the material (such as bamboo, wood, grasses, reeds or other vegetable matter of fibrous nature) containing 30 the same, wherein the extraction of the solubles from the material fed into any digestor is effected by digestion in a semi-continuous, progressive, step-by-step or cascade system, but more particularly wherein the digestion 35 is effected in a generally increasing pressure and free caustic or digesting liquor concentration gradient, or in a series of steps or stages, the digesting liquor concentration and the pressure generally being raised at 40 each stage, from the first treatment of the fresh stock until the digestion is nearly complete, characterized by the digestor liquor activity or concentration in the last stage of digestion, or the composition of the digesting liquor, and, if desired, the pressure also, 45 in the final stage or stages of digestion being modified with the object of avoiding hydrolysis of the cellulose fibre in said last stage or stages.
- 50 The invention also includes a process for separating or extracting cellulose or paper pulp from the material containing the same wherein the extraction of the solubles from the material fed into any digestor is effected 55 in stages by digestion on a semi-continuous, progressive, step-by-step system or on a cascade system, wherein a modification is introduced in that the greatest strength of active alkali is not at the last digestion stage but 60 such greatest strength is at some stage earlier in the digestion, preferably at a lower pressure, and when more of the non-cellulosic material still remains to be removed, in order 65 to prevent or reduce the hydrolysis of

the cellulose fibre in the final stages of digestion.

It may comprise processes such as those referred to above wherein mixed digesting liquors are used, such as caustic and sulphites 70 and/or sulphides (which latter exert a protective action reducing the tendency towards hydrolysis of the cellulose fibres taking place), and the liquors added are proportioned in such a way that hydrolysis is prevented or reduced by having a greater proportion of the protective reagents in the final stage or stages of the digestion.

The invention may comprise such a process 80 wherein mixed digesting liquors are used and wherein the liquor or liquors, of those used, which have the greater retarding effect on the hydrolysis of the cellulose at raised pressures is or are in excess, or form the whole of the liquor, in the final stage or stages of the digestion, the liquor or liquors having a stronger effect in causing hydrolysis being added at 85 a point in the digestion process before the final stage in the digestion is reached and while the fibre still contains a considerable 90 or appreciable proportion of non-cellulosic matter.

It also includes a process wherein mixed caustic liquor and sulphide and/or sulphite liquor are used, but wherein the sulphide or sulphite liquor or liquors is or are used alone or in excess in the final stage or stages of the digestion owing to their retarding effect on hydrolysis of the fibre, but wherein the caustic is added at a point in the digestion before 95 the completion stage, is reached.

The invention may further include a process as described, or as claimed in any of the claims of my application Serial No. 253,310, filed February 10, 1928, and Patent No. 1,690, 100 954, dated November 6, 1928, wherein a mixed digestor liquor is used in a portion at least of the digestion process, and wherein the different digestion liquors are supplied 105 from separate sources with the object that the composition of the said liquor in the different digestion stages may be varied as desired.

In this last process the modification may 110 be introduced in that the whole of the fresh digestion liquor is not added to that digestor which is about to undergo its final digestion, but instead further fresh digestion liquor is added to a digestor in a subsequent stage of 115 the general step-down pressure-liquor-concentration series.

The invention further includes a process 120 wherein the digestor undergoing final digestion at the highest steam pressures has sodium sulphite, or sodium sulphide, or both a sulphite and sulphide, as the digesting liquor, or in which the digesting liquor for the final digestion has a considerable proportion of sulphite or sulphide therein, and wherein into 125 the next digestor in the step-down pressure 130

series, or alternatively, at some other step or period of the digestion, caustic soda is added to make up the strength of the digesting liquor.

5 The invention also includes within its scope the modification whereby in addition to the variations in the digesting liquor composition the pressure in the final stage or portion of the digestion is held steady for a period or is even reduced to below the maximum pressure used in said digesting for the purposes explained.

Having now particularly described and ascertained the nature of my said invention and 15 in what manner the same is to be performed, I declare that what I claim is:—

1. A cascade process for the extraction of cellulose pulp from fibre yielding vegetable material, which comprises treating the material with digester liquor and under pressure in stages in digesters, progressively increasing the pressure and active liquor concentration at each stage until the digestion is nearly complete, and then varying the active liquor concentration in the final stages sufficiently to substantially prevent the hydrolysis of the cellulose fibre in the final stages.

2. A process according to claim 1, wherein the active liquor concentration is reduced in 30 the final stages.

3. A cascade process for the extraction of cellulose pulp from fibre yielding vegetable material, which comprises treating the material under pressure and with mixed caustic 35 and sulphite liquors in stages in a plurality of digestors, progressively increasing the pressure and caustic liquor concentration at each stage until the digestion is nearly complete, and then reducing the proportion of 40 caustic liquor in the final stages to a value sufficient to substantially prevent the hydrolysis of the cellulose fibre in the final stages.

4. A cascade process for the extraction of cellulose pulp fibre yielding vegetable material, which comprises treating the material in stages in digesters under pressure and with a mixed liquor composed of caustic liquor and a liquor having a retarding influence on the hydrolysis of cellulose fibre at 45 raised pressures, progressively increasing the pressure and the caustic liquor concentration until the digestion is nearly complete, and then increasing the proportion of retarding liquor in the final stages until it is in 50 excess of the caustic liquor.

5. A cascade process for the extraction of cellulose pulp from fibre yielding vegetable material, which comprises treating the material in stages in digesters under pressure 55 and with a liquor composed of a mixture of caustic and other liquors supplied from separate sources, progressively increasing the pressure and the concentration of caustic in said liquor at each stage until the digestion is nearly complete, and then varying the

supply of said liquors in the final stages to reduce the proportion of caustic therein to a value sufficient to prevent the hydrolysis of the cellulose fibre in the final stages.

6. A cascade process for the extraction of cellulose pulp from fibre yielding vegetable material, which comprises treating the material in stages in digesters under pressure and with a mixed liquor composed of caustic soda and sodium sulphite, progressively increasing the pressure and the caustic concentration at each stage until the digestion is nearly complete, and then treating the material in the final stages with a liquor composed substantially entirely of sodium sulphite.

7. A cascade process for the extraction of cellulose pulp from fibre yielding vegetable material, which comprises treating the material in stages in digesters under pressure and with a mixed liquor including sodium sulphite, progressively increasing the pressure and adding caustic soda until the digestion is nearly complete, and then increasing the proportion of sodium sulphite until the liquor in the final stages is composed substantially entirely of sodium sulphite.

8. A cascade process for the extraction of cellulose pulp from fibre yielding vegetable material, which comprises treating the material with a mixed liquor and under pressure in stages in digesters, progressively increasing the pressure and active liquor concentration at each stage until the digestion is nearly complete, and then maintaining the pressure constant and reducing the active liquor concentration in the final stages sufficiently to substantially prevent the hydrolysis of the cellulose fibre in the final stages.

In testimony whereof I hereto affix my signature this 11th day of January, 1928.

EDMONDSON SPENCER